



US005556730A

**United States Patent** [19]**Nguyen**[11] **Patent Number:** **5,556,730**[45] **Date of Patent:** **Sep. 17, 1996**

[54] **CHARGE INJECTION BARRIER FOR  
POSITIVE CHARGING ORGANIC  
PHOTOCONDUCTOR**

4,943,501 7/1990 Kinoshita et al. .... 430/67 X  
5,069,993 12/1991 Robinette et al. .... 430/66 X  
5,096,793 3/1992 Osawa et al. .... 430/67 X

[75] Inventor: **Khe C. Nguyen**, Los Altos, Calif.

**FOREIGN PATENT DOCUMENTS**

[73] Assignee: **Hewlett-Packard Company**, Palo Alto, Calif.

2-168262 6/1990 Japan ..... 430/66  
2-146556 6/1990 Japan ..... 430/66  
5-34958 2/1993 Japan ..... 430/66

[21] Appl. No.: **548,348**

*Primary Examiner*—Roland Martin

[22] Filed: **Nov. 1, 1995**

**ABSTRACT****Related U.S. Application Data**

[62] Division of Ser. No. 180,750, Jan. 12, 1994, Pat. No. 5,476,604.

[51] Int. Cl.<sup>6</sup> ..... **G03G 5/09; G03G 5/147**

[52] U.S. Cl. ..... **430/66; 430/67; 430/83;  
430/58; 430/59**

[58] **Field of Search** ..... 430/66,67,83

[56] **References Cited**

**U.S. PATENT DOCUMENTS**

4,923,775 5/1990 Schank ..... 430/66 X

**3 Claims, 7 Drawing Sheets**







FIG. 3



FIG. 4



FIG. 5



FIG. 6



FIG. 7

## DARK DECAY AT THE LAB AMBIENT

EXAMPLES  
FIG. 8

## DARK DECAY AT 70 C

EXAMPLES  
FIG. 9



FIG. 11



FIG. 13



CYCLE  
FIG. 14

## CHARGE INJECTION BARRIER FOR POSITIVE CHARGING ORGANIC PHOTOCONDUCTOR

This application is a divisional application of my prior, utility patent application entitled "CHARGE INJECTION BARRIER FOR POSITIVE CHARGING ORGANIC PHOTOCOCONDUCTOR", Ser. No. 08/180,750, filed Jan. 12, 1994, now U.S. Pat. No. 5,476,604.

### BACKGROUND OF THE INVENTION

#### 1. Technical Field

This invention relates generally to photoconductors for electrophotography. The invention is a positive charging, organic photoconductor material with good speed and improved stability for liquid toner electrophotography. The improved stability is a result of a positive charge injection barrier layer on top of the organic photoconductor material.

#### 2. Related Art

In electrophotography, a latent image is created on the surface of photoconducting material by selectively exposing areas of the charged surface to light. A difference in electrostatic charge density is created between the areas on the surface exposed and unexposed to light. The visible image is developed by electrostatic toners containing pigment components and thermoplastic components. The toners are selectively attracted to the photoconductor surface either exposed or unexposed to light, depending on the relative electrostatic charges of the photoconductor surface, development electrode and the toner. The photoconductor may be either positively or negatively charged, and the toner system similarly may contain negatively or positively charged particles. For laser printers, the preferred embodiment is that the photoconductor and toner have the same polarity, but different levels of charge.

A sheet of paper or intermediate transfer medium is then given an electrostatic charge opposite that of the toner and passed close to the photoconductor surface, pulling the toner from the photoconductor surface onto the paper or intermediate medium, still in the pattern of the image developed from the photoconductor surface. A set of fuser rollers fixes the toner to the paper, subsequent to direct transfer, or indirect transfer when using an intermediate transfer medium, producing the printed image.

The important photoconductor surface, therefore, has been the subject of much research and development in the electrophotography art. A large number of photoconductor materials have been disclosed as being suitable for the electrophotographic photoconductor surface. For example, inorganic compounds such as amorphous silicon (Si), arsenic selenite ( $As_2Se_3$ ), cadmium sulfide (CdS), selenium (Se), titanium oxide ( $TiO_2$ ) and zinc oxide (ZnO) function as photoconductors. However, these inorganic materials do not satisfy modern requirements in the electrophotography art of low production costs, high-speed response to laser diode or other light-emitting-diode (LED), and safety from non-toxicity.

Therefore, recent progress in the electrophotography art with the photoconductor surface has been made with organic materials as organic photoconductors (OPC's). Typically, the OPC's in the current market are of the dual-layer, negative-charging type with a thin charge generation material layer, usually less than about 1 micron ( $\mu m$ ) thick, beneath a thicker charge transport material layer deposited on top of the charge generation layer. However, positive

charging OPC's ((+)OPC's) are preferred for a discharged area developed (DAD) image as in laser printers.

Specific morphologies of phthalocyanine pigment (Pc) powder have been known to exhibit excellent photoconductivity. These phthalocyanine pigments have been used as a mixture in polymeric binder matrices in electrophotographic photoconductors, deposited on a conductive substrate.

The photoconductivity of the phthalocyanine pigment may be used to formulate the (+)OPC. Currently, known (+)OPC's may be classified as follows:

5 1. Single layer (+)OPC—Type I (see FIG. 1). The Pc is uniformly distributed throughout a relatively thick binder layer on a conductive substrate. Photons striking the upper surface of the layer generate positive and negative charges there. The generated negative charges neutralize positive charges established on the surface of the layer by the biasing corotron, discharging them. The generated positive charges travel through the bulk of the layer towards negative charges established by the biasing corotron at the conductive substrate.

10 20 In these Type I single-layer photoconductors, then, there is no need to add charge transport molecules, nor to have a separate charge transport layer. The phthalocyanine pigment content may be in the range of about 5-30 wt. %, high enough to perform both charge generation and charge transport functions, with the binder content being in the range of about 95-70 wt. %.

15 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945

Other layers may be added to the OPC. To improve the transfer efficiency of the toner, for example, the top surface of the OPC may be overcoated with a low surface adhesion material. This type of overcoat layer is known as a release layer. See, for example, U.S. Pat. No. 4,923,775.

The charging characteristics of the photoconductor is the most important factor for high image quality in the conventional xerographic copiers or printers. Unfortunately, the charging characteristics of the photoconductor may be easily affected by electrical or chemical contamination, and/or by physical damage to the surface incurred during the printing process. The deterioration of the charging characteristics, thus, is frequently the cause of poor print quality. Many commercially available photoconductors experience deterioration of surface charging due to the effect of mechanical wear. However, the most common cause of charge instability in the positive charging photoconductor is not only mechanical wear or damage. Instead, the instability of the surface charge is exhibited as a decrease in charge acceptance along with an increase in dark decay electrical properties of the photoconductor after repeated cycles. Charge instability is also increased at operating temperatures above room temperature.

The mechanism of the charge instability in the (+)OPC, so far, is not well understood. It is expected that the surface of the (+)OPC is more chemically vulnerable to the operating conditions such as corona charging, ozone attack, humidity, heat, etc. Especially, this phenomenon is more prominent for the (+) OPC's classified as Types I, II, III and IV above mentioned. In these (+) OPC's configurations, the hole transport components such as pigment or hole transport molecules are directly exposed to the Corona during charging. It is suspected that these (+) OPC's (Types I, II, III and IV but not V) above are more likely to exhibit deteriorated charge characteristics due to surface charge injection into the bulk of the (+)OPC. This phenomenon is more critical in (+)OPC's than in some well known inorganic photoconductors, such as amorphous selenium, CdS, etc.

Therefore, the main object of this invention is to provide a charge injection barrier for the (+) OPC which exhibits stable electrical properties, including charge acceptance, dark decay and photodischarge, in a high cycle, high severity electrophotographic process. It is known to provide a charge injection preventing layer for (+) OPC's, such as a layer of SiO<sub>2</sub> (silica) embedded in a polymer matrix. With such kind of heterogeneous phase, however it was found that it scatters the light from the exposure source and reduces the writing incident energy. Furthermore, a severe ghosting phenomenon is frequently observed using such kinds of heterogeneous barrier materials. The ghosting image phenomenon is associated with the light fatigue effect of the photoconductive device. This phenomenon generates the residual image from the previous imaging cycle into the new print. So, it is another objective of this invention to provide a charge injection preventing layer which does not cause the ghosting and the reduced contrast image.

Presently, the (+) OPC with the added release layer discussed above to enhance toner transfer efficiency is used only in single run applications. The incorporation of the release layer on the outer layer of the OPC does not appear to contribute to surface charge stability. In some cases, it is noticed that the release layer even adversely affects the OPC's charge stability. This adverse affect is believed to be the result of leakage of the catalyst used to cross-link the release layer into the bulk of the OPC. (See U.S. Pat. No. 4,923,775.)

Another goal of the present invention is to provide the solution of the organic coating barrier for the crosslinkable

top coat including poly siloxanes and the other type of the crosslinking binders. In this case, the organic coating barrier is expected to stop the photoconductor poisoning from the leaking of the catalyst or the chemicals from the top coating of polysiloxanes.

Thus, the barrier layer for the surface of the (+)OPC in the present invention is basically comprised of selected molecules or moieties which are capable of prohibiting the injection of the unwanted positive charge from the surface of the photoconductor into the bulk of the photoconductor without stopping the migration of the negative charge from the photoconductor bulk toward the surface. Such kinds of highly functional chemical species must be embedded uniformly in a selected crosslinkable polymer matrix. The selected materials and process must not cause any optical perturbation to the photoresponse process of the photoconductor, and must be robust enough in the operating environment to withstand high humidity and high temperature.

#### DISCLOSURE OF THE INVENTION

To solve this OPC stability problem, a charge injection barrier layer is placed on top of the OPC. The barrier may have 2 layers—1, an electron withdrawing layer on top of the OPC;—2, an electron donating layer on top of the electron withdrawing layer. This formulation resulted in a long-life OPC with more than 50,000 good cycles at high severity test conditions.

The barrier layer comprises: 1. a crosslinked polymer binder; 2. a charge injection prohibiter molecule, and, optionally; 3. an electron withdrawing molecule.

The crosslinkable binder material for the barrier layer may be selected from

a. Reactive hydroxy group containing polymers which exhibit:

1. reactivities with —SiOH, —SiH, —Si(OR)3;
  2. self-crosslinking by thermal cure;
  3. reactivities with thermoset binders including melamine resin, poly diisocyanate, epoxy resin, phenolic resin, polyimide, alkyd resin, poly siloxanes, polyfluorosiloxanes, etc.; and
  4. reactivities with functional groups such as aldehydes, dialdehydes, poly-ols, alcohols, anhydrides, etc.
- b. Reactive anhydride containing polymers such as styrene-maleic anhydrides; and
- c. Mixtures of (a) and (b) above.

The positive charge injection prohibiting (CIP) molecule is an electron donating molecule which has a functional group which forms hydrogen bonds with, for example, the lone pair of N atoms of the phthalocyanine pigment compounds. This way, the prohibitor molecule restricts the generation of free positive charge from the phthalocyanine pigment, especially under heat or electric field. These functional groups for the prohibitor molecule are —OH (hydroxy), —NH<sub>2</sub>, —NH or —N<(amino).

Preferably, the barrier layer may also contain an electron acceptor and/or electron transporter molecule, known as an electron withdrawing molecule (EWM). These molecules have the —C=O (carbonyl), —Cl, —Br, —I, —F (halogen), —NO<sub>2</sub> (nitro), —CN (cyano), —OH (hydroxy), —SO<sub>2</sub> (sulfuryl/sulfonyl) or —COOH (carboxylic) functional groups.

From practicing this invention, one can produce an OPC with not only long life during continuous use, but also long shelf life and long on-again/off-again operation life.

## BRIEF DESCRIPTION OF THE DRAWINGS

FIGS. 1-5 are schematic, cross-sectional views of current OPC constructions.

FIGS. 6 and 7 are schematic, cross-sectional views of several embodiments of the invention.

FIGS. 8-14 are graphic results of the results of some of the worked Examples.

## BEST MODE FOR CARRYING OUT INVENTION

10

Referring to FIGS. 6 and 7, there are depicted several schematic, cross-sectional views of several embodiments of the invention. An OPC is provided with a conductive substrate, and a photoconductor layer on top of the substrate. A charge injection barrier layer is placed on top of the photoconductor layer. The charge injection barrier layer may contain a separate electron withdrawing layer on top of the OPC, and a separate electron donating layer on top of the electron withdrawing layer. Also, an optional release layer may be placed on top of the injection barrier layer. Also, other layers, not shown, which are commonly used in OPC's may be used, such as, for example, charge blocking layers, anti-curl layers, overcoating layers, and the like.

The conductive substrate and photoconductor layer on top of it may be made of conventional materials and assembled by conventional techniques.

In general, the cross-linkable polymeric binder for the charge injection barrier is selected from:

a. Reactive hydroxy group containing polymers which exhibit:

1. reactivities with  $-\text{SiOH}$ ,  $-\text{SiH}$ ,  $-\text{Si(OR)}_3$ ;
2. self-crosslinking by thermal cure;
3. reactivities with thermoset binders including melamine resin, poly diisocyanate, epoxy resin, phenolic resin, polyimide, alkyd resin, poly siloxanes, polyfluorosiloxanes, etc.; and
4. reactivities with functional groups such as aldehydes, dialdehydes, poly-ols, alcohols, anhydrides, etc.

For this invention, the binder resin of the charge injection barrier layer is preferably cross-linked polyvinyl alcohol (PVA) and its co-polymers.

Polyvinyl alcohol (PVA) has the following formula:



The co-polymer of PVA and polymethylmethacrylate has the following formula:



The co-polymer of PVA and polystyrene has the following formula:



The co-polymer of PVA and fluoro polymer has the following formula:



Polyvinyl butyral (PVB) has the following formula:



where

$$q=50-95 \text{ mol \%}$$

$$r=0.5-15 \text{ mol \%}, \text{ and}$$

$$s=5-35 \text{ mol \%}.$$

The PVA or PVB cross-linking may be effected simply by heating them to between about 150°-300° C. for about 2 hours. Other ways of cross-linking, for example, e-beam, UV or X-ray radiation, may also achieve results similar to those obtained with heat. The cross-linking reaction may be due to the  $-\text{OH}$  groups and the  $-\text{O}-$  groups from different locations on the same PVA or PVB polymer chain, or from different PVA or PVB chains, interacting to form bridge bonds.

Besides PVA or PVB, these crosslinkable polymers include phenolic resin and its copolymers, silanol terminated polysiloxanes and its derivatives, hydroxylated polystyrene and its derivatives, hydroxylated polyesters, hydroxylated polycarbonates, cellulose and its derivatives, for example, nitro cellulose, butyl cellulose and ethyl cellulose, and polyvinyl acetals, which have the following formula:



Where R=alkyl, alkoxy, amine groups, aminoalkyl, cyano  $-\text{CN}$ , halogen (Cl, Br, I, F), nitro  $-\text{NO}_2$ , hydroxy  $-\text{OH}$ , aryl and arylalkyl with substituent groups  $-\text{NO}_2$ ,  $-\text{CN}$ ,  $-\text{OH}$ , halogens, amine, heterocyclic groups, etc.,

b. Reactive anhydride containing polymers such as styrene-maleic anhydrides; and

c. Mixtures of (a) and (b) above.

The crosslinking reaction of the above-mentioned polymers may be carried out, in general, by a thermal curing process, irradiation curing process, including e-beam cure, UV cure, or x-ray cure, and moisture cure. The crosslinking reaction may take place between portions of the polymer itself, called self-crosslinking, without adding any crosslinking aids. Or, a crosslinking aid may be added to accelerate the crosslinking reaction. These crosslinkers, in this case, may be selected from:

Alkoxy silanes having the general chemical structure



or



where  $\text{R}_1, \text{R}_2, \text{R}_3$ =alkyl, allyl, aryl, with or without the conventional substituent groups;

Aldehydes, alcohols, carboxylic acid anhydrides; and

Thermoset binders as mentioned above.

A second crosslinking binder may be added to the above crosslinkable binders. These second binders are called co-crosslinkers, and may be selected from the conventional thermoset binders such as epoxy, melamine resin, unsaturated polyesters, polydiisocyanate, alkyd resin, polyimides, etc. Molecular weights for the binders may vary from about 20,000 to about 1,500,000.

Also, the positive charge injection barrier comprises a positive charge injection prohibiting (CIP) molecule. The positive charge injection prohibitor molecule is an electron donating molecule which has a functional group which forms hydrogen bonds with, for example, the lone pair of N atoms of the phthalocyanine pigment compounds. This way, the prohibitor molecule restricts the generation of free positive charge from the phthalocyanine pigment, especially under heat or electric field. These functional groups for the prohibitor molecule are —OH (hydroxy), —NH<sub>2</sub>, —NH, or —N=(amino). I expect a similar mechanism to be operative with the other pigments besides the phthalocyanine ones.

Positive charge injection prohibiting compounds may be from the specific amino compounds of the general formulas:



or from the specific hydroxy or mercapto compounds of the general formulas:



Where, for formulas 9-18 above: 45

R<sub>1</sub>, R<sub>3</sub>, R<sub>5</sub>=alkyl, alkoxy, allyl, aryl, with and/or without the following substituent groups: —NO<sub>2</sub>, —CN, —OH, —SH, —SO<sub>2</sub>, —SOCl<sub>2</sub>, —S, —C=O, —COOR, —CHO, —Cl, —Br, —I, —F;

R<sub>2</sub>=hydrogen, alkyl, alkoxy, aryl with and/or without the following substituent groups —NO<sub>2</sub>, —CN, —OH, —SH, —SO<sub>2</sub>, —SOCl<sub>2</sub>, —C=O, —CHO—COOR, —Cl, —Br, —I, —F;

A=heterocyclic compounds selected from the following groups: 55



60



(20)



(21)



(22)



(23)



(24)



(25)



(26)



(27)



(28)



(29)

**9**  
-continued



m,n=1,2 . . . 5.

For example, some CIP molecules may be:

1. Aminobenzimidazole
2. 4-Amino-1-benzylpiperidine
3. 1-Amino-2-(dimethyl amino) fluorene
4. 1-Amino-2,6-dimethylpiperidine
5. 2-Amino-4,6-dimethylpyridine
6. 3-Amino-5,6-dimethyl-1,2,4-diazine
7. 4-Amino-3,5-di-2-pyridyl-4H-1,2,4-triazole
8. 3-Amino-9-ethylcarbazole
9. 2-(2-Amino ethyl)-1-methylpyrrole
10. 2-(2-Amino ethyl)-1-methylpyrrolidine
11. 1-(2-Amino ethyl) pyridine
12. 1-(2-Amino ethyl) piperazine
13. 1-(2-Amino ethyl) piperidine
14. 1-Amino-4-(2-Hydroxy ethyl) piperidine
15. 2-Amino-9-hydroxy fluorene
16. 3-Amino-5-hydroxy pyrazole
17. 2-Amino-3-hydroxy pyridine
18. 5-Amino iso quinoline
19. 4-Amino-2-mercaptop pyrimidine
20. 2-Amino-5-mercaptop-1,2,4-triazole
21. 6-Amino-5-nitroso-2-thiouracil
22. 3-Amino propyl triethoxy silane
23. 3-Amino propyl trimethoxy silane
24. (Cyclohexyl amino methyl) methyl diethoxy silane
25. (Cyclohexyl amino methyl) dimethylethoxy silane
26. N,N-Diethyl amino trimethyl silane
27. 2,2,4,4,6,6-Hexamethyl cyclo trisilazane



**10**

28. Octamethyl cyclo tetrasilazane (30)
- 5 29. (R)-N<sub>1</sub>-phenethyl-N<sup>1</sup>-trietoxy silyl propylurea (31)
- 10 30. Tetrakis (dimethyl amino) silane (32)
- 15 31. 1,1,4,4-Tetramethyl-1,4-Bis (N,N-dimethyl amino)-disilethylene (33)
- 20 32. N-[3-(Triethoxy silyl)propyl]-4,5-dihydro imidazole (34)
- 25 33. Trimethoxy silyl propyl diethylenetriamine (35)
- 30 34. 1-Trimethyl silyl-1,2,4-triazole (36)
- 35 35. 1,3,5-Trimethyl-1,3,5-trivinyl cyclo trisilazane (37)
- 40 36. Tris (cyclo hexyl amino) methyl silane (38)
- 45 37. Tris (dimethyl amino) phenyl silane (39)
- 50 38. N,O-Bis (trimethyl silyl) hydroxylamine (40)
- 55 39. N-(2-Amino ethyl)-3-amino propyl methyl dimethoxy silane (41)
- 60 40. Diethyl (trimethyl silyl methyl) phosphonate (42)
- 65 41. (Tinuvin® 328)
42. 2-(2'-Hydroxy-3',5'-di-tert-amyl phenyl) benzotriazole (43)
43. (Tinuvin® 770)

## 11

- Bis(2,2,6,6-tetramethyl-4-piperidyl) sebacate  
 43. (Tinuvin® 144)  
 Bis(1,2,2,6,6-pentamethyl-4-piperidinyl) (3,5-di-tert-butyl-4-hydroxybenzyl) butyl propane dioate  
 44. (Tinuvin® 292)  
 Bis(1,2,2,6,6-penta methyl-4-piperidinyl) sebacate  
 45. (Irganox® 259)  
 1,6-Hexamethylene bis (3,5-di-tert-butyl-4-hydroxy cinnamate  
 46. (Irganox® 1010)  
 Tetrakis [methylene (3,5-di-tert-butyl-4-hydroxy hydro cinnamate] methane  
 47. (Irganox® 1035)  
 Thiodiethylene bis (3,5-di-tert-butyl-4-hydroxy hydro cinnamate  
 48. (Irganox® 1076)  
 Octadecyl 3,5-di-tert-butyl-4-hydroxy hydro cinnamate  
 49. AgeRite Resin D® powder  
 Polymerized 1,2-dihydro-2,2,4-trimethyl quinoline

Preferably, the positive charge injection barrier layer may also contain an electron acceptor and/or electron transporter molecule, known as an electron withdrawing molecule (EWM).

Examples of electron withdrawing molecules are:

- 1) phthalic anhydride
- 2) dinitrophenol
- 3) 2-methylanthraquinone
- 4) 2, 7-dinitrofluorene
- 5) 2, 7-dinitrofluorenone
- 6) (2R)-(+)-Glycidyl tosylate.

If the charge injection barrier layer itself has separate layers, the electron acceptor/transporter molecules (EWM) are predominantly in the sensitizing layer.

The ratio of electron acceptor molecule to electron donor molecule is between about 100/1-1/100. If the charge injection barrier layer is in one combined layer, the electron accepting and electron donating molecules may be combined into one bipolar molecule, for example, methyl hydantoin, di-nitro aniline, di-nitro-fluoro aniline, or di-nitro-biphenyl amine. When the charge injection prohibiting molecule and the electron withdrawing molecule are in the same molecule, the general chemical structure of the molecule is

A-R-D (43),

where A represents the electron withdrawing part of the molecule, selected from the electron withdrawing functional groups:  $-\text{NO}_2$ ,  $-\text{CN}$ ,  $=\text{C}=\text{O}$ ,  $-\text{SO}_x \text{ X}=1, 1.5, 2, 3, 3.5$  and 4,  $-\text{S}$ ,  $-\text{OR}$ ; R=alkyl, allyl, aryl; and D represents the charge injection prohibiting part of the molecule,

Examples of A-R-D molecules are:

- 1) 2,3-Pyridinedicarboxylic anhydride
- 2) Dinitrofluoro aniline
- 3) 4,5-Dicyanoimidazole
- 4) 2,6-Dichloropurine
- 5) Maleimide
- 6) Methyl hydantoin
- 7) O-benzoic sulfimide
- 8) 2-(4-Aminophenyl)-6-methylbenzothiazole
- 9) 2-Amino-5-(4-nitrophenylsulfonyl) thiazole
- 10) N,N-Dimethylindoaniline.

The optional overcoating release layer may comprise organic polymers such as polydimethylsiloxane (PDMS) and its derivatives, including fluoro alkyl substituted PDMS, silanol terminated PDMS, methyl hydrogen siloxane terminated PDMS, vinyl terminated PDMS, etc., or inorganic polymers that are electrically insulating or slightly semi-

## 12

conductive. This overcoating layer may range in thickness from about 0.1  $\mu\text{m}$  to about 8  $\mu\text{m}$ , and preferably from about 3  $\mu\text{m}$  to about 6  $\mu\text{m}$ . An optimum range of thickness is from about 3  $\mu\text{m}$  to about 5  $\mu\text{m}$ .

- 5 The process of making the barrier layer for this invention is defined by a uniform mixture of the required components: reactive hydroxy binder, charge injection prohibiter, optional crosslinker, optional second crosslinker (co-crosslinking binder), and optional electron withdrawing molecules into the appropriate solvent and then coating of the solution on the top of the photoconductor. The coating process may be done by a number of different procedures including dip coating, ring coating, spray coating, or hopper coating, etc.
- 10 The drying process for the barrier layer 3 is basically comprised of two steps: solvent eliminating step which may be carried out at room temperature or at the boiling point of the used solvent, and the crosslinking step which causes the crosslinking reaction of the crosslinkable binder. The crosslinking step may be done at different temperatures including lab ambient such as moisture cure, or at elevated temperature from 80° C. -200° C., such as thermal cure. The thickness of the coating can be varied from 0.001  $\mu\text{m}$  to 20  $\mu\text{m}$ . The most desirable range of the thickness is between 0.01  $\mu\text{m}$  to 5  $\mu\text{m}$ .
- 15 This kind of the surface protection material for the photoconductor can be applied for any types of photoconductor which is comprised of photoconductive pigment embedded in a polymeric binder, including ZnO, CdS, phthalocyanine-binder or thin film photoconductor such as Se, amorphous Si, or multi layer OPC, especially, positive charging photoconductors.
- 20 The following EXAMPLES will clarify the uniqueness of the invention.

## EXAMPLE 1

## Preparation of the Photoconductor

16 g of x—H<sub>2</sub>Pc, 84 g of polycarbonate (Mobay Chemical, Makrolon™), 900 g of dichloromethane, 2000 g of Zr beads, 3 mm diameter, were milled together in a ceramic container using a ball mill for 48 hrs. The blue suspension, after being separated from milling media, was applied with a doctor blade on an Al/Mylar™ substrate. The coating thickness was about 7  $\mu\text{m}$  after being dried at 80° C. for 4 hrs.

## EXAMPLE 2

## Preparation of the Barrier Layer

|                                              |         |
|----------------------------------------------|---------|
| Polyvinylbutyral (B98, Monsanto Chemical)    | 65% wt. |
| Amino propyl triethoxysilane (Aldrich Chem.) | 25% wt. |
| Phthalic anhydride                           | 10% wt. |

60 were dissolved in Isopropyl alcohol (IPA) to achieve 5 wt. % solids. The solution was coated on the surface of an OPC formulated in EXAMPLE 1, using a doctor blade in order to achieve a coating thickness of 1  $\mu\text{m}$ . The coating layer was dried at the lab ambient for 1 hr. and then baked in an oven at 140° C. for another 1 hr.

## 13

## EXAMPLE 3

## Preparation of the Top Coat

|                                                  |           |
|--------------------------------------------------|-----------|
| Poly dimethyl siloxane (Sylloff 23, Dow Corning) | 100 part  |
| Catalyst 23A                                     | 1 part    |
| Heptane                                          | 1900 part |

were dissolved together. The solution was coated on the top of an OPC formulated in EXAMPLE 1 using a doctor blade in order to achieve a thickness of 3  $\mu\text{m}$  after being dried at 135° C. for 10 minutes.

## EXAMPLE 4

## Preparation of OPC Having Both the Barrier Layer and the Top Coat

The OPC bearing the protection layer of EXAMPLE 2 was overcoated with the solution described in EXAMPLE 3 and by the same procedure as Example 3 to form a triolayer OPC comprised of OPC layer, barrier layer and the top coat.

All of these OPC samples were tested by being wrapped around a well grounded A1 drum of 180 mm diameter. The A1 drum was inserted into a laser printing test mechanism developed at Hewlett-Packard Co. For a life test, in each cycle, the OPC sample was exposed to a corona charger, then, a 780 nm laser scanned with polygon mirror to produce 2 mW output, and then to a LED eraser. The corona charger was set to a grid voltage of +600 V, and a corona current of 450  $\mu\text{A}$ . The surface potential of the OPC is detected using an electrostatic charge probe (Trek Model 362) placed between the corona charger and the area of laser exposure. The drum rotation speed was set at 3 inches per second. In order to test the OPC performance at high temperature, a sheet heater was inserted inside of the drum, and the drum was monitored and controlled by a thermocouple placed closely to the surface of the photoconductor and connected to the heater.

## Test 1. Dark Decay

The dark decay characteristics of the photoconductors were tested by measuring the surface potential decay during 2 minutes after stopping the corona power supply.

## Test 2. Life Test

The life of the photoconductors were tested by measuring the surface potential at the beginning of each cycle (charging, laser exposing, LED erasing).

## Results

FIG. 8—dark decay at the lab ambient of each EXAMPLE 1, 2, 3, and 4.

FIG. 9—dark decay at 70° C. of each EXAMPLE 1, 2, 3 and 4.

FIG. 10—10K cycle life at the lab ambient of each EXAMPLE 1, 2, 3 and 4.

FIG. 11—10K cycle life at 70° C. of each EXAMPLE 1, 2, 3 and 4.

From FIG. 8 and FIG. 9, one can see that the barrier layer significantly reduces the dark decay, especially at high temperature such as 70° C., revealing the effective prevention of surface charge injection.

From FIG. 10 and FIG. 11, it is also observed that the photoconductor life is significantly improved when the barrier layer was used for either case, with or without top coat of polysiloxanes. It should be noted that the top coat of polysiloxanes, for example, has been known as a protection

## 14

layer coating in the prior art. However, in these experiments, I observed the surface charge deterioration in the photoconductor sample having the top coat of polysiloxanes. In this case, the instability of the surface charge (EXAMPLE 3) can be explained as the chemical poisoning of the photoconductive layer, and may be due to the leakage of the catalyst of the crosslinking reaction from the polysiloxanes coating into the bulk of the OPC. The improvement of the surface charge stability in EXAMPLE 4 reveals that the barrier coating of EXAMPLE 2 has effectively prevented the leakage of the catalyst from the top coat of polysiloxanes.

## EXAMPLE 5

## Preparation of the Electron Withdrawing Layer

|                                                     |            |
|-----------------------------------------------------|------------|
| Poly vinyl butyral B98, Monsanto Chemical           | 60 parts   |
| Dinitrophenol (Electron Withdrawing Molecule (EWM)) | 20 parts   |
| Pyridine dicarboxylic acid anhydride (crosslinker)  | 20 parts   |
| Isopropyl Alcohol (IPA)                             | 4000 parts |

The whole mixture was dissolved completely by stirring, and coated on the top of an OPC formulated as in EXAMPLE 1, using a doctor blade. The coating thickness was about 0.5  $\mu\text{m}$  after being dried at 135° C. for 1 hr.

## EXAMPLE 6

## Preparation of the Charge Injecting Prohibiter Layer

|                                                 |          |
|-------------------------------------------------|----------|
| Poly vinyl butyral (B98, Monsanto Chemical)     | 1 part   |
| Amino propyl alkoxy silane (Z6020, Dow Corning) | 20 part  |
| Isopropyl alcohol (IPA)                         | 819 part |

The whole mixture was dissolved completely by stirring, and coated on the top of an OPC formulated as in EXAMPLE 5 using a doctor blade. The coating layer was dried in air for 30 minutes and at 80° C. for 20 minutes. The coating thickness was about 0.5  $\mu\text{m}$ .

## EXAMPLE 7

The top coat solution described in EXAMPLE 3, was used to coat the top of the OPC formulated in EXAMPLE 6, by the same coating procedure as in EXAMPLE 3. This four-layer OPC exhibited an excellent life at 70° C. exceeding 60,000 cycles as indicated in FIG. 12.

## EXAMPLE 8

## Preparation of a Multi-Layer Positive Charging Photoconductor (I)

4 g of hole transport molecule (44)



## 15

and 6 g of polycarbonate (Makrolon<sup>TM</sup>) were dissolved in 90 g of dichloromethane (DCM). The solution was coated on an aluminum/mylar substrate using a doctor blade so that the coating thickness became about 15  $\mu\text{m}$  after being dried at 100° C. for 2 hrs. This coating layer performs as a charge transport layer (CTL).

Next, 3 g of x—H<sub>2</sub>P<sub>c</sub>, 27 g of hole transport molecule (44) above described, 70 g of polycarbonate (Makrolon<sup>TM</sup>), and 500 g of dichloromethane (DCM) were milled together using a ball milling procedure with 5 mm ceramic balls as 10 milling media. The milling time was 40 hrs. The solution, after milling, was coated on the top of the charge transport layer above-mentioned, using a doctor blade to achieve a thickness of 6  $\mu\text{m}$  after being dried at 130° C. for 2 hrs. This layer performs as a charge generation layer (CGL).

## EXAMPLE 9

## Preparation of a Barrier Protection Layer for the Multi-Layer Photoconductor of Example 8.

First, the electron withdrawing layer described in Example 5 was overcoated on the top of the multi-layer photoconductor of Example 8.

Second, the charge injecting prohibitor layer was overcoated on the electron withdrawing layer, using the same manner described in Example 6.

Finally, the top coat solution described in Example 3 was coated on the top of the charge injecting prohibitor layer, using the same procedure described in Example 3. For 30 comparison, the life test results of Example 8 (bare photoconductor) and of Example 9 (protection layer photoconductor) are illustrated in FIG. 13.

## EXAMPLE 10

## Preparation of a Multilayer Positive Charging (+) Photoconductor II.

3 g of x—H<sub>2</sub>P<sub>c</sub> pigment, 1.5 g of polyester (Vylon 200<sup>TM</sup> Toyobo) and 100 g of dichloromethane (DCM) were milled 40 together using 5 mm ceramic beads as milling media, in a ceramic pot and on a roll miller. The system was milled for 48 hrs.

The solution was coated on Al/Mylar flexible substrate using a doctor blade to achieve a thickness of 0.1  $\mu\text{m}$  after being dried at 100° C. for 40 minutes. This forms a charge generation layer (CGL).

Next, 4 g of an electron transport molecule (45)



prepared by a method described in *J. Org. Chem.*, 50, 3297 (1985), by F. Menger and D. Carnahan, 6 g of polycarbonate (Lexan<sup>TM</sup>—General Electric) and 90 g of dichloromethane were mixed together by stirring until a completely dissolved 65 solution was achieved. This solution was overcoated on the top of the charge generation layer above mentioned, using a

## 16

doctor blade so that a thickness of 15  $\mu\text{m}$  was achieved after being dried at 100° C. for 4 hrs.

## EXAMPLE 11

## Preparation of a Barrier Layer for the Multi Layer Photoconductor of Example 10.

The (+) OPC described in Example 10 was overcoated first with a barrier layer (described in Example 6); and second with the top coat of poly dimethyl siloxane (described in Example 3)

The comparison of results for the bare photoconductor (Example 10) and full construction photoconductor (Example 11) is illustrated in FIG. 14.

While there is shown and described the present preferred embodiment of the invention, it is to be distinctly understood that this invention is not limited thereto but may be variously embodied to practice within the scope of the following claims.

What is claimed is:

1. An organic photoconductor for electrophotography comprising:

a conductive substrate;

an organic photogenerating layer on top of said conductive substrate, said photogenerating layer comprising a photogenerating pigment component uniformly dispersed in an organic binder material, and a charge transporting component also uniformly dispersed in said organic binder material; and

a charge injection barrier layer on top of said photogenerating layer, said injection barrier layer comprising: a cross-linked organic binder material comprising polyvinyl alcohol (PVA), and

a positive charge injection prohibiting molecule selected from the group consisting of amino compounds having the general formulas:



or from the group consisting of hydroxy or mercapto compounds having the general formulas:



Where, for formulas 9-18 above:

R<sub>1</sub>, R<sub>3</sub>, R<sub>5</sub>=alkyl, alkoxy, allyl, aryl, with and/or without the following substituent groups: —NO<sub>2</sub>, —CN, —OH, —SH, —SO<sub>2</sub>, —SOCl<sub>2</sub>, —S, =C=O, —COOR, —CHO, —Cl, —Br, —I, or —F;

R<sub>2</sub> is hydrogen, alkyl, alkoxy, or aryl with and/or without the following substituent groups —NO<sub>2</sub>, —CN, —OH,

**17**

—SH, —SO<sub>2</sub>, —SOCl<sub>2</sub>, —S, —C=O, —COOR,  
—CHO, —Cl, —Br, —I, or —F;

A=heterocyclic compounds selected from the group consisting of:

5  
(19)10  
(20)15  
(21)20  
(22)25  
(23)30  
(24)35  
(25)40  
(26)45  
(27)**18**

-continued

(27)



(28)



(29)



(30)



(31)



(32)



and m,n=1,2 . . . 5.

2. The photoconductor of claim 1 which also comprises an overcoat layer on top of the injection barrier layer.

3. The photoconductor of claim 2 wherein the overcoat layer comprises polydimethylsiloxane (PDMS).

\* \* \* \* \*